

Aug. 10, 1926.

1,595,731

J. V. QUIGLEY

DIFFERENTIAL COAL FLOTATION

Filed May 24, 1922



INVENTOR

John Vir Quigley  
BY Williams & Hitchcock  
ATTORNEYS

## UNITED STATES PATENT OFFICE.

JOHN VIE QUIGLEY, OF ALAMEDA, CALIFORNIA, ASSIGNOR TO MINERALS SEPARATION NORTH AMERICAN CORPORATION, OF NEW YORK, N. Y., A CORPORATION OF MARYLAND.

## DIFFERENTIAL COAL FLOTATION.

Application filed May 24, 1922. Serial No. 563,215.

This invention relates to the froth-flo-  
tation concentration of coal-bearing materials  
and as herein described is applied to the se-  
lective flotation of bituminous coal so as to  
produce from a single lot of coal one or  
more concentrates which are relatively rich-  
er in carbon and have a lower content of  
sulphur than the untreated coal. In the  
form of the invention herein disclosed the  
bituminous coal is first agitated in the ab-  
sence of any added agent to produce a coal-  
bearing froth, which is then separated.  
There is then added to the pulp containing  
the remainder of the coal, an agent such as  
petroleum oil, and the pulp is further agi-  
tated to produce a second coal-bearing froth.  
The two froths are separately collected and  
are found to vary quite widely from each  
other in character.

It is found that certain "bright-coal" in-  
gredients are preferentially separated in the  
first froth, produced in the absence of added  
agent. These ingredients may have an ash  
approximately of the composition of the  
original plant ash, and this first froth,  
carrying these ingredients, contains much  
less ash than the original coal. The con-  
centrate thus obtained also contains much  
less sulphur than the original coal.

It is found that the second froth, produced  
with the addition of an agent, contains a  
relatively large proportion of other coal  
ingredients dull in appearance to the naked  
eye.

The coal of the first froth is usually of  
great purity and well adapted for use in  
arts demanding a coal of this character, and  
is particularly free from substances detri-  
mental to the production of metallurgical  
coke. The coal of the second froth is about  
of the richness of the original coal, or  
slightly richer. The tailings are largely  
composed of ash and contain a considerable  
part of the sulphur.

The examples herein described were car-  
ried out in a subaeration machine of the kind  
shown in sectional side view in the accom-  
panying drawing.

This machine has an agitation chamber 1,  
of rectangular cross-section, provided with  
an agitator 2 turning near the bottom of  
the chamber and carried by a shaft 3, which

is journaled in overhead bearings 4 and 5,  
and has a driving pulley 6, at the top, and  
is supported just below the pulley by a suit- 55  
able thrust bearing 7.

To form a froth, the agitator 2 is driven  
in the proper direction at a suitable speed  
and air is thereby drawn in through a bot- 60  
tom pipe 9, suitably connected by a U-exten-  
sion to an upright pipe 10, extending above  
the level of the pulley in the chamber 1  
and provided with a valve 11 to control the  
admission of air beneath the agitator 2. A 65  
suitable baffle 12 is located above the agi-  
tator 2, and is shown as formed of inter-  
secting metal sheets 13 and 14, set at right  
angles to each other.

Alongside of the agitation chamber 1 is  
formed a spitzkasten 18 and the wall 17 70  
between the agitation chamber and the spitz-  
kasten terminates at the top below the pulp  
level, and provides communication at the  
bottom between the agitation chamber and  
spitzkasten, thus permitting the pulp to flow 75  
over the top of this partition into the spitz-  
kasten and to flow downward and back from  
the spitzkasten into the agitation chamber.

A draining opening 24, closed by a plug  
25, is located in the bottom of the agitation 80  
chamber.

The following are examples of procedures  
embodying my invention:

1. A coal from the United States Coal and  
Coke Company taken from mine No. 40 at 85  
Phillipi, West Virginia, was crushed dry  
to pass through a 10-mesh Tyler screen. It  
was then thoroughly mixed with water to  
form a pulp and was agitated for 10 min- 90  
utes to form a first coal-bearing froth con-  
centrate A, which was then removed. This  
first concentrate contained a large propor- 95  
tion of bright coal. There was then added  
one pound per ton of a light stove oil made  
by the California Petroleum Company from  
California crude having an asphalt base.

The oil had a gravity of 30 to 35 Baumé, a  
flash point of 160°, a fire point of 190°, con-  
tained a high percentage of kerosene oil and  
no more than 4% of asphalt. When agi- 100  
tated with this oil for 15 minutes the re-  
mainder of the pulp yielded a second coal-  
bearing froth concentrate B. This second  
concentrate contained a large proportion of

dull coal. The results are shown in the following table:

| 5             | Wt. | % Wt. | % Ash. | % S.  | % Recovery |
|---------------|-----|-------|--------|-------|------------|
| Heads-----    | 506 | 100.0 | 14.20  | 4.62  |            |
| Conc. A-----  | 85  | 16.8  | 3.5    | 0.99  |            |
| Conc. B-----  | 356 | 70.4  | 8.6    | 1.98  |            |
| Tailings----- | 65  | 12.8  | 59.0   | 23.21 | 99.8       |

10 2. A coal from mine No. 3 of the same company at the same place was similarly crushed and then reground wet in a ball mill for 5 minutes, resulting in approximately 100 mesh grinding. It was similarly agitated in the same machine for 12 minutes yielding a first coal-bearing froth concentrate A, largely bright coal, which was collected for a period of 12 minutes. There 15 was then added to the remainder of the pulp 1.25 pounds per ton of the same light stove oil and agitation was continued for 13 minutes producing a second coal-bearing froth concentrate B, largely dull coal. The results are shown in the following table:

| 25            | Wt. | % Wt. | % Ash. | % S. | % Recovery |
|---------------|-----|-------|--------|------|------------|
| Heads-----    | 697 | 100.0 | 8.83   | 0.75 |            |
| Conc. A-----  | 320 | 48.0  | 3.0    | 0.55 |            |
| Conc. B-----  | 235 | 48.0  | 7.4    | 0.66 |            |
| Tailings----- | 42  | 6.0   | 65.6   | 3.08 | 99.9       |

30 3. A coal from the Woodward Iron Company, Woodward, Alabama, was crushed dry to pass a 10-mesh standard Tyler screen, then mixed with water to form a pulp and agitated in a subaeration machine for 12 minutes without any added reagent. During this time a first coal-bearing froth concentrate A, largely bright coal, was collected. There 35 was then added to the remainder of the pulp 1.2 pounds of the same light stove oil and the pulp was reagitated and a second coal-bearing froth concentrate B, largely dull coal, was collected for 13 minutes. The results are shown in the following table:

| 45            | Wt. | % Wt. | % Ash. | % S. | % Recovery |
|---------------|-----|-------|--------|------|------------|
| Heads-----    | 660 | 100.0 | 17.72  | 1.26 |            |
| Conc. A-----  | 215 | 32.6  | 2.8    | 0.83 |            |
| Conc. B-----  | 316 | 47.9  | 6.6    | 0.88 |            |
| Tailings----- | 129 | 19.5  | 70.0   | 2.92 | 96.8       |

50 4. A coal from the Westmoreland Coal and Coke Company, Legonia, Pennsylvania, was crushed dry to pass a 10-mesh standard Tyler screen and then reground in a ball mill for 5 minutes to produce approximately 100-mesh material. The coal was then made into a pulp and agitated in the subaeration machine without any reagent for 13 minutes. During this time a first coal-bearing froth concentrate A, largely bright coal, was collected. The same light stove oil was then

55 added at the rate of one pound per ton and the pulp was reagitated for a period of 12 minutes, producing a second coal-bearing froth concentrate B, largely dull coal, which was collected. The results are shown in the following table:

| 60            | Wt. | % Wt. | % Ash. | % S. | % Recovery |
|---------------|-----|-------|--------|------|------------|
| Heads-----    | 599 | 100.0 | 15.13  | 1.29 |            |
| Conc. A-----  | 286 | 47.7  | 7.8    | 0.99 |            |
| Conc. B-----  | 272 | 45.4  | 16.0   | 1.32 |            |
| Tailings----- | 41  | 6.9   | 60.0   | 3.19 | 99.7       |

65 It will be observed that in every case a larger proportion of the ash went into the tailings and that a substantially larger proportion of the sulphur went into the tailings than was retained in the concentrates.

70 It will be noted that this method of coal concentration produces a means for economically recovering the coal and at the same time dividing it into portions each having valuable properties and each especially suited for special purposes in the arts.

75 That is, according to the present invention, one concentrate is separated consisting of superior coal which has been floated in a froth without the addition of added mineral-frothing agent or oil, and thereafter another concentrate is separated consisting of inferior coal which was floated as a froth in the presence of suitable added agent or oil, while the final tailings are usually discarded. No claim is broadly 80 made herein to the concentration of coal by froth-flotation wherein the process is begun in the absence of any added mineral-frothing agent or oil and is completed by the aid of such an agent or oil or both. The latter invention is described and claimed in the application of William Truran, Serial No. 563,841, filed concurrently herewith.

85 It is obvious that in the embodiment of this invention in the concentration of coal-bearing materials to which it is applicable the agents used and the proportions in which they are added and the details of operation will be adjusted to the particular requirements in each instance as determined by test and trial as is well known in this art.

90 I claim:—

95 1. The process of concentrating coal-bearing material which consists in agitating and aerating a pulp of the suitably ground material to produce a coal-bearing froth without addition of an agent and separating and segregating the froth, then adding an agent to the depleted pulp and subjecting the 100 depleted pulp to further agitation and aeration to form a second coal-bearing froth, and separating and segregating the second froth.

105 2. The process of concentrating coal-bear-

ing material which consists in agitating and aerating a pulp of the suitably ground material to produce a coal-bearing froth without addition of an agent and separating and 5 segregating the froth, then adding an oily agent to the depleted pulp and subjecting the depleted pulp to further agitation and aeration to form a second coal-bearing froth, and separating and segregating 10 the second froth.

3. The process of concentrating coal-bearing material which consists in agitating and aerating a pulp of the suitably ground material to produce a coal-bearing froth without 15 addition of an agent and separating and segregating the froth, then adding a petroleum oil to the depleted pulp and subjecting the depleted pulp to further agitation and aeration to form a second coal-bearing 20 froth, and separating and segregating the second froth.

4. The process of separating bright coal from dull coal which consists in agitating and aerating a pulp of finely divided suitable coal to produce a bright-coal-bearing 25 froth without addition of an agent and separating and segregating the froth, then adding an agent to the depleted pulp and subjecting the depleted pulp to further

agitation and aeration to form a dull-coal-bearing froth, and separating and segregating the second froth.

5. The process of separating bright coal from dull coal which consists in agitating and aerating a pulp of finely divided suitable coal to produce a bright-coal-bearing froth without addition of an agent and separating and segregating the froth, then adding an oily agent to the depleted pulp and subjecting the depleted pulp to further 40 agitation and aeration to form a dull-coal-bearing froth, and separating and segregating the second froth.

6. The process of separating bright coal from dull coal which consists in agitating and aerating a pulp of finely divided suitable coal to produce a bright-coal-bearing froth without addition of an agent and separating and segregating the froth, then adding a petroleum oil to the depleted pulp and subjecting the depleted pulp to further agitation and aeration to form a dull-coal-bearing froth, and separating and segregating the second froth.

In testimony whereof, I have affixed my 55 signature to this specification.

JOHN VIR QUIGLEY.